

# United States Patent Office

**3,573,050**

Patented Mar. 30, 1971

1

3.573.050

**COLOR PHOTOGRAPHIC LAYERS COMPRISING  
NON-DIFFUSIBLE 5 - HYDROXYCOUMARANS  
AS STABILIZING COMPOUNDS**

AS STABILIZING COMPOUNDS  
Kent C. Brannock, Kingsport, Tenn., and Gregory J. Lestina, Rochester, N.Y., assignors to Eastman Kodak Company, Rochester, N.Y.  
No Drawing. Filed Feb. 27, 1969, Ser. No. 803,080  
Int. Cl. G03c 1/84, 1/40

Int. Cl. G03C 17/07, 17/40  
U.S. Cl. 96—84 16 Claims

## 16 Claims

## **ABSTRACT OF THE DISCLOSURE**

Nondiffusible 5-hydroxycoumaran stabilizer compounds which have either a substituted amino group or an alkoxy group substituted on the carbon atoms in the 2 position are advantageously incorporated in hydrophilic colloid layers of photographic elements in which color photographic dye images are to be stored for viewing. The stabilizer compounds protect dye images against the fading effects of prolonged exposure to light.

This invention relates to photography, photographic materials including color photographic materials containing dye image stabilizing agents, and methods for improving the stabilities of dyes in photographic materials.

The formation of dye images by the chromogenic development of silver halide photographic materials, involving the coupling reaction of oxidized primary aromatic amino developing agents with coupling compounds to form indophenol, indamine, azomethine, phenoxazine, phenazine, and similar dyes, is well known. In this system, the subtractive color process of color formation is ordinarily used and the image dyes customarily formed are cyan, magenta, and yellow, which are the colors that are complementary to the primary colors, red, green and blue, respectively. Usually phenolic couplers (i.e., phenols and naphthols) are used to form the cyan dye image; pyrazolone or cyanoacetyl couplers are used to form the magenta dye image; and acylacetamide or dibenzoylmethane couplers are used to form the yellow dye image.

In these color photographic systems, the color-forming coupler may be applied in a developer solution or incorporated in the light-sensitive photographic emulsion layer or in another dye-image-forming layer, so that, during development, it is available to react with oxidized color developing agent formed as the result of latent image development.

The dye images formed in such processes are not indefinitely stable to ultraviolet radiation so that under rigorous viewing or display conditions involving, for example, long periods of exposure to sunlight, or other ultraviolet radiant illumination, the dyes may fade, resulting in deterioration in the quality of the picture.

Increases in the stability of indophenol, indoaniline, and azomethine dyes to ultraviolet radiation have been achieved by the use of a variety of agents which can be added to the emulsion in processing, or more conveniently, in manufacture. Lestina and Reckhow describe the use of dinuclear 6-hydroxy chroman stabilizers in photographic elements in U.S. Ser. No. 452,889, filed May 3, 1965 now U.S. Pat. No. 3,432,300. The need remains for still other stabilizers that will further enhance the resistance of these dyes to actinic light.

It is therefore an object of our invention to provide novel photographic elements containing dyes and/or dye-forming compounds, and 5-hydroxycoumaran stabilizer compounds to increase the stability of the dyes against ultraviolet and visible light radiation.

Another object of our invention is to provide novel image dye stabilizing agents which do not form highly

24

colored oxidation products in the processing baths, e.g., bleach baths, etc., used in color photographic processing.

Another object of our invention is to provide novel color photographic image-forming layers comprising hydrophilic colloid film-forming binders containing finely particulate dispersions of solutions of our 5-hydroxycoumaran stabilizing agents.

It is a further object to provide such layers also containing couplers.

0 A further object is to provide novel dispersions of our  
5-hydroxycoumaran stabilizing agents which can be in-  
corporated in silver halide emulsion layers without ad-  
verse emulsion effects.

It is a still further object of our invention to provide novel processed color photographic layers containing dye images in association with the 5-hydroxycoumaran stabilizing agents of our invention.

These and other objects will be apparent from a consideration of the following specification and claims.

20 These and other objects are accomplished according to our invention by providing hydrophilic colloid layers for the storage of dye images that are stabilized against the effects of prolonged exposure to light by the incorporation of a nondiffusible 5-hydroxycoumaran, such as, a 25 2-amino-5-hydroxycoumaran and a 2-alkoxy-5-hydroxycoumaran. Our stabilizing compounds are particularly advantageous for the stabilization of indophenol dye images, indoaniline dye images, azomethine dye images and azo dye images that are stored in hydrophilic colloid layers 30 for viewing. These dye images are either formed as non-diffusible dye images in the hydrophilic colloid layer containing our stabilizer compound or are formed as diffusible dye images in another hydrophilic colloid layer and transferred to a receiving layer containing a hydrophilic colloid layer with our stabilizer compound. Our 35 invention provides valuable technical advances.

Our nondiffusible 5-hydroxycoumaran stabilizing compounds include those represented by the formula:



wherein R<sub>1</sub> represents hydrogen, an alkyl group, preferably an alkyl group having from 1 to 22 carbon atoms (e.g., methyl, ethyl, isopropyl, butyl, t-butyl, cyclohexyl,

(e.g., methyl, ethyl, isopropyl, butyl, t-butyl, cyclohexyl, 50 octyl, t-octyl, dodecyl, octadecyl, docosyl, etc.) and the atoms necessary to complete with  $R_2$  a fully hydrogenated hydrocarbon ring of 4 to 7 atoms, preferably 5 to 6 atoms in the ring (e.g., cyclobutane, cyclopentane, cyclohexane, cycloheptane, etc.);  $R_2$  represents an alkyl group having 55 from 1 to 22 carbon atoms as described for  $R_1$  and the atoms necessary to complete with  $R_1$  a fully hydrogenated hydrocarbon ring of 4 to 7 atoms, preferably 5 to 6 atoms in the ring (e.g., cyclobutane, cyclopentane, cyclohexane, cycloheptane, etc.).

hydrocarbon ring of 4 to 7 atoms, preferably 5 to 6 atoms in the ring (e.g., cyclobutane, cyclopentane, cyclohexane, cycloheptane, etc.);  $R_3$  represents hydrogen, an alkyl group, preferably having from 1 to 22 carbon atoms, such as have been described for  $R_1$  and an alkoxy group having from 1 to 22 carbon atoms (e.g., methoxy, propoxy, t-butoxy, hexoxy, 2-methylpentylxyloxy, dodecoxyl, octadecoxyl, docosoxyl, etc.;  $R_4$  represents hydrogen, or

octadecoxy, docosoxy, etc.;  $R_4$  represents hydrogen, an alkyl group having from 1 to 22 carbon atoms and preferably a branched chain alkyl group (e.g., methyl, isopropyl, t-butyl, 2-methylpentyl, 2,2-dimethylpentyl, t-octyl, dodecyl, octadecyl, docosyl, etc.), an alkoxy group having from 1 to 22 carbon atoms as described for  $R_3$ , and the atoms necessary to complete with  $R_5$  a 5, 6 or 7 membered carbocyclic ring, such as, a cyclopentane ring (e.g., cyclopentane methylcyclopentane, methoxycyclopentane, etc.).

tane, etc.), a cyclohexane ring (e.g., cyclohexane, ethylcyclohexane, ethoxycyclohexane,  $\omega$ -hydroxyhexylcyclohexane, etc.) and a cycloheptane ring (e.g., cycloheptane, ethylcycloheptane, methoxycycloheptane,  $\omega$ -hydroxybutoxycycloheptane, etc.);  $R_5$  represents hydrogen, an alkyl group having from 1 to 22 carbon atoms as described for  $R_1$ , a mononuclear aryl group (e.g., phenyl, tolyl, ethylphenyl, etc.), an alkoxy group having from 1 to 22 carbon atoms as has been described for  $R_3$ , and the atoms necessary to complete with  $R_4$  a 5, 6 or 7 membered carbocyclic ring, such as, a cyclopentane ring (e.g., cyclopentane, methylocyclopentane, methoxycyclopentane, etc.), a cyclohexane ring (e.g., cyclohexane, ethylcyclohexane, ethoxycyclohexane,  $\omega$ -hydroxyhexylcyclohexane, etc.) and a cycloheptane ring (e.g., cycloheptane, ethylcycloheptane, methoxycycloheptane,  $\omega$ -hydroxybutoxycycloheptane, etc.);  $Z$  represents a



group or a  $-OR_8$  group;  $R_6$  represents an alkyl group, preferably an alkyl group of from 1 to 22 carbon atoms (e.g., methyl, isopropyl, *t*-butyl, 2-methylpentyl, 2,2-dimethylpentyl, *t*-octyl, dodecyl, octadecyl, docosyl, 2,3-pentenyl, 3,4-pentenyl, 2-hydroxyethyl, 2-chloroethyl, 2-carboxyethyl, 3-sulfopropyl, 2-cyanoethyl, 2-nitroethyl, 4-nitrobutyl, cyclobutyl, cyclopentyl, cyclohexyl, 2-methylcyclohexyl, cycloheptyl, etc.), an aryl group, such as, a phenyl group (e.g., phenyl, *p*-tolyl, *o*-tolyl, *o*-ethylphenyl, *p*-isopropylphenyl, etc.), a naphthyl group (e.g.,  $\alpha$ -naphthyl, 2-methyl- $\alpha$ -naphthyl,  $\beta$ -naphthyl, etc.), a heterocyclic group having from 4 to 7 and preferably 5 to 6 atoms in the heterocyclic ring (e.g., pyridyl, quinolyl, thiazolyl, benzothiazolyl, naphthothiazolyl, oxazolyl, benzoxazolyl, imidazolyl, benzimidazolyl, etc.), and the atoms necessary to complete with  $R_7$  a heterocyclic ring having from 4 to 7 atoms and preferably 5 to 6 atoms in the ring (e.g., piperidino, morpholino, thiamorpholino, pyrrolidinyl, etc.);  $R_7$  represents an alkyl group preferably an alkyl group of from 1 to 22 carbon atoms (e.g., methyl, isopropyl, *t*-butyl, 2-methylpentyl, 2,2-dimethylpentyl, *t*-octyl, dodecyl, octadecyl, docosyl, 2,3-pentenyl, 3,4-pentenyl, 2-hydroxyethyl, 2-chloroethyl, 2-carboxyethyl, 3-sulfopropyl, 2-cyanoethyl, 2-nitroethyl, 4-nitrobutyl, cyclobutyl, cyclopentyl, cyclohexyl, 2-methylcyclohexyl, cycloheptyl, etc.), an aryl group, such as, a phenyl (e.g., phenyl, *p*-tolyl, *o*-tolyl, *o*-ethylphenyl, *p*-isopropylphenyl, etc.), a naphthyl group, e.g.,  $\alpha$ -naphthyl, 2-methyl- $\alpha$ -naphthyl,  $\beta$ -naphthyl, etc.), a heterocyclic group having from 4 to 7 and preferably 5 to 6 atoms in the heterocyclic ring (e.g., pyridyl, quinolyl, thiazolyl, benzothiazolyl, naphthothiazolyl, oxazolyl, benzoxazolyl, imidazolyl, benzimidazolyl, etc.), and the atoms necessary to complete with  $R_6$  a heterocyclic ring having from 4 to 7 atoms and preferably 5 to 6 atoms in the ring (e.g., piperidino, morpholino, thiamorpholino, pyrrolidinyl, etc.); and  $R_8$  represents an alkyl group having from 1 to 22 carbon atoms as has been described for the alkyl group under  $R_6$  and  $R_7$ .

Included among the compounds of Formula I that are used advantageously according to our invention are the following typical compounds:

- (1) 6 - *t*-butyl-3,3-dimethyl-5-hydroxy-2-morpholinocoumaran



(2) 6 - *t* - butyl-3,3-dimethyl-2-(N'-ethoxycarbonyl-N-piperazino)-5-hydroxycoumaran



(3) 6 - *t* - butyl-3-butyl-5-hydroxy-2-piperadino coumaran

(4) 3,3-dimethyl - 5 - hydroxy-2-(N-methylanilino)-6-*t*-octylcoumaran

(5) 5-hydroxy - 2 - (N-butylanilino)-3-methyl-6-*t*-octylcoumaran



(6) 3,3-dimethyl - 5 - hydroxy-(N-methylanilino)-6-*t*-octoxycoumaran

(7) 6 - *t* - butyl-3,3-dimethyl-5-hydroxy-2-(N-methylanilino)coumaran

(8) 6 - *t* - butyl-3,3-dimethyl-2-(3-ethoxycarbonylpiperidino)-5-hydroxycoumaran

(9) 3,3-dibutyl - 5 - hydroxy-2-(N-methylanilino)-6-*t*-octylcoumaran

(10) 6 - *t* - butyl-3,3-dibutyl-5-hydroxy-2-(N-methylanilino)coumaran

(11) 3-butyl - 3 - ethyl-5-hydroxy-2-(N-methylanilino)-6-*t*-octylcoumaran

(12) 3,3-dimethyl - 5 - hydroxy-2-(N-methyl-N-hexylamino)-6-*t*-octylcoumaran

(13) 3,3-dimethyl - 5 - hydroxy-2,6-*t*-octyl piperidinocoumaran

(14) 6 - *t* - butyl-3,3-dimethyl-5-hydroxy-2-(N-methyl-N-octadecylamino)coumaran

(15) 2-(N-anilino) - 6 - *t* - butoxy-5-hydroxy-3,3,4-trimethylcoumaran

(16) 7 - *t* - butyl-3,3-dimethyl-4-ethoxy-5-hydroxy-2-(N-methylanilino)coumaran

(17) 6-*t*-butyl-3,3-dimethyl-5-hydroxy-2-(N-methylanilino)-7-phenylcoumaran

(18) 6-*t*-butyl-3,3-dimethyl-7-ethoxy-5-hydroxy-2-(N-methylanilino)coumaran

(19) 3,3-dimethyl-2-(N,N-dimethylamino)-5-hydroxy-6,7,8,9-tetrahydrobenzocoumaran

(20) 6-*t*-butyl-3,3-dimethyl-2-ethoxy-5-hydroxycoumaran

(21) 3-butyl-2-ethoxy-3-ethyl-5-hydroxy-

5-*t*-octylcoumaran

(22) 3,3-dimethyl-2-ethoxy-5-hydroxy-6-*t*-octylcoumaran

(23) 2-butoxy-6-*t*-butyl-3,3-dimethyl-5-hydroxycoumaran

(24) 6-*t*-butyl-3,3-dimethyl-5-hydroxy-2-octadecyl-

oxycoumaran

(25) 6-*t*-butyl-3,3-dimethyl-2-docosoxy-5-hydroxy-

coumaran

(26) 6-*t*-butyl-3,3-dimethyl-5-hydroxy-2-(2-methyl-

pentoxy)coumaran

Our stabilizing agents are advantageously used to improve the stability of the indophenol, indoaniline and azomethine dyes, such as, those produced by chromogenic development, the azo dyes produced in well-known diazo-type elements, and dyes produced in well-known silver-dye-bleach elements and the dyes used in dye transfer, dye imbibition and dye diffusion transfer systems. Our stabilizing agents are advantageously incorporated in the layer in which the dye image will be stored after image formation; this is either the layer in which a nondiffusible dye image is formed or the layer to which a diffusible dye image is transferred, such as, the image-receiving layer of a receiving sheet in a dye-transfer system, a dye-imbibition system or a dye-diffusion transfer system. The specific

method used to form the indophenol, indoaniline, azomethine, or azo dye is not important since any of the well-known image-forming elements and processes are used advantageously.

Our stabilizers are particularly efficacious in protecting dyes produced by chromogenic development of any of the well-known 5-pyrazolone couplers used in photography for magenta dye formation. Typical magenta dyes are those produced by color development of couplers described in U.S. patents, such as, 2,600,788, 2,725,292, 2,908,573, 3,006,759, 3,062,653, 3,152,896, 3,311,476 and Young U.S. application Ser. No. 458,455, filed May 24, 1965, now U.S. Pat. No. 3,419,391, which couplers are herein incorporated by reference.

Cyan dye-forming couplers of such U.S. patents as 2,474,293, 2,725,292, 2,895,826, 2,908,573 produce cyan dyes upon chromogenic development that are advantageously stabilized against light exposure by our stabilizing compounds.

Yellow dye-forming couplers of U.S. Pat. 2,908,573 produce yellow dyes that are made less subject to the fading effects of prolonged exposure to light by the presence of our stabilizing compounds.

Our stabilizing agents are incorporated alone or together with a color-forming coupler in a dye image-forming layer of a color photographic element. A useful method of dispersing our stabilizing compounds is that described for dispersing couplers in Mannes et al. U.S. Pat. 2,304,939, issued Dec. 15, 1942; Jelley et al. U.S. Pat. 2,322,027, issued June 15, 1943, etc., in which high-boiling organic solvents are used to dissolve the material. Other applicable methods are described in Vittum et al. U.S. Pat. 2,801,170, and Fierke et al. U.S. Pat. 2,801,171, both issued July 30, 1957, and Julian U.S. Pat. 2,949,360, issued Aug. 16, 1960, in which low-boiling or water-soluble organic solvents are used with high-boiling solvent.

In these methods of dispersion our stabilizing agents can be contained in the same dispersion with nondiffusing couplers, or in a separate dispersion, and the couples can optionally be dispersed directly in the emulsion. High-boiling solvents useful in dispersing the 5-hydroxycoumaran stabilizer compounds of our invention include di-n-butylphthalate, benzylphthalate, triphenyl phosphate, tri-cresyl phosphate, diphenyl mono-p-tert-butylphenyl phosphate, monophenyl di-p-tert-butylphenyl phosphate, diphenyl mono-o-chlorophenyl phosphate, monophenyl di-o-chlorophenyl phosphate, tri-p-tert-butylphenyl mono(5-tert-butyl-2-phenylphenyl)phosphate, 2,4-di-n-amylphenol, 2,4-di-t-amylphenol, N,N-diethylauramide, etc.

The low-boiling or water-soluble organic solvents which can be used to advantage with the high-boiling solvents are disclosed in patents, such as Fierke et al. U.S. Pat. 2,801,171, and Vittum et al. U.S. Pat. 2,801,170, both issued July 30, 1957, and Julian U.S. Pat. 2,949,360, issued Aug. 16, 1960, etc.

The organic solvents include:

(1) Low-boiling, substantially water-insoluble organic solvents, such as, methyl, ethyl, propyl, and butyl acetates, isopropyl acetate, ethyl propionate, sec-butyl alcohol, ethyl formate, butyl formate, nitromethane, nitroethane, carbon tetrachloride, chloroform, etc., and

(2) Water-soluble organic solvents, such as methyl isobutyl ketone,  $\beta$ -ethoxyethyl acetate, tetrahydrofurfuryl adipate, Carbitol acetate (diethyleneglycol monoacetate), methoxytriglycol acetate, methyl Cellosolve acetate, acetyl acetone, diacetone alcohol, butyl Carbitol, butyl Cellosolve, methyl Carbitol, methyl Cellosolve, ethylene glycol, diethylene glycol, dipropylene glycol, acetone, methanol, ethanol, acetonitrile, dimethylformamide, dioxane, etc.

Combinations of two or more of the new and improved dye-stabilizing agents of our invention may be used. These agents may also be used in combination with other addenda into the same dispersion, for example, other stabilizing agents, antistain agents, e.g., ballasted hydroquinones,

phenolic antioxidants, etc. The selection of the specific stabilizer compound and the concentration used in each layer of a multilayer film can be varied over a wide range, and will depend on the improvement in resistance to fading required for each of the image dyes in the respective layers.

Any of the well-known primary aromatic amino color-forming silver halide developing agents such as the phenylenediamines, e.g., N,N-diethyl-p-phenylenediamine hydrochloride, N-monomethyl-p-phenylenediamine hydrochloride, N,N-dimethyl-p-phenylenediamine hydrochloride, 2-amino-5-diethylaminotoluene hydrochloride, 2-amino-5-(N-ethyl-N-laurylamo)toluene, N-ethyl-N- $\beta$ -(methylsulfonamido)ethyl-3-methyl-4-aminoaniline sulfate, N-ethyl-N-( $\beta$ -methylsulfonamidoethyl)-4-aminoaniline, 4-(N-ethyl-N- $\beta$ -hydroxyethyl)aminoaniline, etc., the p-aminophenols and their substitution products where the amino group is unsubstituted, e.g., 2,6-dichloro-4-amino-15 phenol, 2-bromo-p-aminophenol, 2,6-diido-4-aminophenol, 4-aminophenol, etc., may be used to develop photographic coatings containing our stabilizers. Various other materials may be included in the developer solutions depending upon the particular requirements, for example, 20 image-forming couplers competing couplers, antifoggants, hardeners, an alkali metal sulfite, bisulfite, alkaline buffer salts, bromide, iodide, etc., and the thickening agents used in viscous developer compositions. A typical developer solution is given in Example 1 but does not limit the 25 invention.

Our stabilizers are incorporated in hydrophilic colloid layers intended for the storage of photographic dye images, such as, a receiving sheet for receiving a diffusible transferred dye image or a dye-image forming layer containing a light-sensitive material such as silver halide (e.g., silver chloride, silver bromide, silver iodide, silver chlorobromide, silver chlorobromoiodide, silver bromoiodide, etc.), a light-sensitive diazo compound (as in diazo-type 30 material), etc.

Hydrophilic colloids used to advantage in the image layers include any of the hydrophilic colloids used in image-forming layers and in receiving layers, such as gelatin, and gelatin derivatives, casein and other proteinaceous colloids, hydrophilic cellulosic derivatives, e.g., 35 carboxymethyl cellulose, alginates, synthetic resins, e.g., polyvinyl alcohol, copoly(ethylacrylate, acrylic acid) polyvinyl pyrrolidone, etc. Some colloids used to advantage are polyvinyl alcohol or a hydrolyzed polyvinyl acetate as described in U.S. Pat. 2,286,215, a far hydrolyzed cellulose ester, such as cellulose acetate hydrolyzed to an acetyl content of 19-26%, as described in U.S. Pat. 2,327,808, a water-soluble ethanolamine cellulose acetate as described in U.S. Pat. 2,322,085, a polyacrylamide having a combined acrylamide content of 40 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 90

such receiving sheets containing our stabilizer compounds, they exhibit marked improvement in light stability.

Usually emulsions containing our stabilizer compounds are coated on photographic supports in the form of multi-layer color photographic elements wherein at least three differently sensitized emulsion layers are coated over one another on the support. Usually the support is coated in succession with a red-sensitive layer, a green-sensitive layer, and a blue-sensitive layer either with or without a Carey Lea filter layer between the blue-sensitive and green-sensitive layers. The three differently color sensitized layers may be arranged in any other order over one another that is desirable; however, the Carey Lea filter layer (i.e., yellow colloidal silver) would not be put over the blue-sensitive layer. Preferably, these light-sensitive layers are arranged on the same side of the support.

In general, our stabilizing agents are used in quantities ranging from 0.25 mole to 20 moles of stabilizer per 1 mole of coupler used (or per 1 mole of dye produced). The preferred range is from 1 mole to 5 moles of stabilizer per mole of coupler (or per mole of dye produced).

The following examples are included for a further understanding of our invention.

#### EXAMPLE 1

Six single layer coatings are made on a paper support of gelatino silver halide emulsions containing 80 mg./ft.<sup>2</sup> of magenta dye-forming coupler No. 6 of U.S. Pat. 3,062,653 (i.e., 1 - (2 - chloro-4,6-dimethylphenyl)-3-{3-[ $\alpha$  - (3 - pentadecylphenoxy)-butyramido]benzamido}-5-pyrazolone), 80 mg./ft.<sup>2</sup> of coupler solvent tricresylphosphate, 320 mg./ft.<sup>2</sup> of gelatin, and 160 mg./ft.<sup>2</sup> of silver, and the amount of addenda indicated in Table I.

TABLE I

|                 | Additional<br>coupler<br>solvent | Compound | Amount                  |
|-----------------|----------------------------------|----------|-------------------------|
| Coating number: |                                  |          |                         |
| 1, control      | None                             | None     | None                    |
| 2               | 40 mg./ft. <sup>2</sup>          | A        | 40 mg./ft. <sup>2</sup> |
| 3, control      | None                             | None     | None                    |
| 4               | 40 mg./ft. <sup>2</sup>          | B        | 40 mg./ft. <sup>2</sup> |
| 5, control      | None                             | None     | None                    |
| 6               | 40 mg./ft. <sup>2</sup>          | X        | 40 mg./ft. <sup>2</sup> |

Compound A is 7 - t - butyl - 2,2 - dimethyl - 6 - hydroxy-4-isopropylchromanol (of French Pat. 1,478,141)

Compound B is 7 - t - butyl - 2,2,4 - trimethyl - 6 - hydroxychromanol (of French Pat. 1,478,141)

Compound X is 6 - t - butyl - 2,2 - dimethyl - 5 - hydroxy-coumaran (of U.S. Pat. 2,535,058)

The coatings are exposed with a 1B intensity scale sensitometer and processed to color negatives using the following process.

|                         | Minutes |
|-------------------------|---------|
| Develop (formula below) | 10      |
| Kodak F-5 fixing bath   | 5       |
| Water wash              | 5       |
| Bleach (ferricyanide)   | 5       |
| Water wash              | 5       |
| Kodak F-5 fixing bath   | 5       |
| Water wash              | 10      |
| Dry                     |         |

#### Developer formula:

Benzyl alcohol—4 ml.  
Sodium hexametaphosphate—0.5 g.  
Sodium sulfite, desiccated—2.0 g.  
Sodium hydroxide—0.16 g.  
4-amino-3-methyl-N-ethyl-N- $\beta$ -(methanesulfonamido) ethylaniline sesquisulfate hydrate—5.0 g.  
Sodium carbonate monohydrate—50.0 g.  
Sodium bromide—0.2 g.  
Water to 1 liter  
pH to 10.75

An area having a magenta dye density of 1.2 is identified in each of the processed coatings which are then subjected to a 10 day northlight fading test (SANS, i.e., simulated average north sky light equivalent to 120,000 foot candle hours). The magenta dye loss at the identified areas having an original density of 1.2 is determined and listed in Table 2.

TABLE 2

|    | Coating No.: | Percent loss in<br>magenta dye density |
|----|--------------|----------------------------------------|
| 1  | -----        | 47                                     |
| 2  | -----        | 6                                      |
| 3  | -----        | 39                                     |
| 4  | -----        | 7                                      |
| 15 | 5            | 58                                     |
|    | 6            | 41                                     |

The data show that compound X is unacceptable as a stabilizer for the magenta dye. From these data it is unexpected that our compounds would be good stabilizers.

#### EXAMPLE 2

Six single layer gelatinous coatings containing a pre-formed magenta dye are made on a support. The coatings have the following compositions:

Dye—33 mg./ft.<sup>2</sup>  
Tricresyl phosphate—165 mg./ft.<sup>2</sup>  
Stabilizer compound indicated in Table 3—15<sup>-4</sup> mole/ft.<sup>2</sup>  
Gelatin—733 mg./ft.<sup>2</sup>  
30 Triisopropylnaphthalene sulfonate—33 mg./ft.<sup>2</sup>  
Saponin—25 mg./ft.<sup>2</sup>

The magenta dye is prepared by reacting the coupler, 1 - (2 - chloro - 4,6 - dimethylphenyl) - 3 - {3 - [ $\alpha$  - (3 - pentadecylphenoxy)butyramido] - benzamido} - 5 - pyrazolone dissolved in tricresyl phosphate with the oxidized form of color developing agent, N - ethyl -  $\beta$  - methanesulfnoamidoethyl - 3 - methyl - 4 - aminoaniline sulfate. The coatings are subjected to SANS light fading test described in Example 1 but for 3 weeks. The stabilizer and the loss in magenta dye density (from an area of the dye image having an original magenta dye density of 1.2) are listed in Table 3.

TABLE 3

|                 | Stabilizing agent | Magenta<br>dye <sup>1</sup> |
|-----------------|-------------------|-----------------------------|
| Coating number: |                   |                             |
| 1               | None, control     | 1.21                        |
| 2               | Compound No. 1    | 0.14                        |
| 3               | Compound No. 2    | 0.16                        |
| 4               | Compound No. 7    | 0.14                        |
| 5               | Compound No. 8    | 0.14                        |
| 6               | Compound No. 15   | 0.20                        |

<sup>1</sup> Density loss from 3 weeks SANS exposure.

45 55 The data show that our stabilizer compounds produce up to an 88% improvement in the stability of the preformed magenta dye compared to the control when subjected to the 3 weeks SANS test.

Similar results are obtained when Example 2 is repeated using magenta dyes produced from the magenta coupler and the oxidized form of other well-known color developing agents including those disclosed herein previously. Similar results are obtained when Example 2 is repeated using any of the other well-known magenta dye-forming couplers with the oxidized form of any of the well-known color-developing agents described herein previously.

#### EXAMPLE 3

70 70 Four single layer gelatinous silver halide emulsion coatings containing the magenta dye-forming coupler, 1-(2-chloro - 4,6 - dimethylphenyl) - 3 - {3 - [ $\alpha$  - (3 - pentadecylphenoxy)butyramido] - benzamido} - 5 - pyrazolone are made on a paper support. The gelatinous silver bromoiodide emulsion is prepared as described by Trivelli

and Smith in the Photographic Journal, page 330, May 1939. The coatings have the following compositions:

TABLE 4

Coupler (identified above)—50 mg./ft.<sup>2</sup>  
 Tricresyl phosphate—50 mg./ft.<sup>2</sup>  
 Stabilizer (as indicated in Table 5)—equimolar to coupler  
 Gelatin—440 mg./ft.<sup>2</sup>  
 Triisopropylnaphthalene sulfonate—20 mg./ft.<sup>2</sup>  
 Saponin—15 mg./ft.<sup>2</sup>

The coatings are dried and given 1/2 second exposure on a 1B intensity scale sensitometer, followed by color processing at 75° F. as follows:

|                     | Min. |
|---------------------|------|
| Color development   | 6    |
| Stop-fix bath       | 3    |
| Wash                | 2    |
| Ferricyanide bleach | 4    |
| Wash                | 3    |
| Hardening fix       | 3    |
| Wash                | 8    |
| Buffer (stabilizer) | 3    |

The color developer is a conventional color developer solution containing benzyl alcohol, sodium sulfite, the color developing agent, N - ethyl -  $\beta$  - methanesulfonamidoethyl - 3 - methyl - 4 - aminoaniline sulfate and an alkali to give a pH of about 10. A conventional stop-fix bath containing sodium thiosulfate, sodium sulfite, acetic acid, boric acid and potassium alum is used for the stop-fix step and for the hardening fix steps in the process. A conventional alkali metal ferricyanide-bromide bleach bath is used, and a conventional aqueous citric acid stabilizer bath having a pH of 3.5 is used in the process. An area having a magenta dye density of about 1.2 is identified on each processed coating before exposing them to a 3 weeks SANS fading test. The results are summarized in the following table.

TABLE 5

| Coating number: | Stabilizer     | 3 weeks<br>SANS<br>magenta dye<br>density loss |      |
|-----------------|----------------|------------------------------------------------|------|
|                 |                | None, control                                  | 1.00 |
| 1               | Compound C     | 0.52                                           |      |
| 2               | Compound No. 4 | 0.25                                           |      |
| 3               | Compound No. 7 | 0.36                                           |      |

The results show that our stabilizer Nos. 4 and 7 produce a substantial improvement in the stability of the magenta dye formed by color development in coating Nos. 3 and 4 compared to coating No. 2 containing prior art stabilizer 2,2,4-trimethyl-6-hydroxy-7-t-octylchroman (compound No. 7 of French Pat. 1,478,141) for the 3 weeks SANS test.

## EXAMPLE 4

Example 3 is repeated using magenta dye-forming 5-pyrazolone couplers 1 through 12 of U.S. Pat. 2,600,788 in place of the coupler used in Example 3. The results are similar to those obtained in Example 3.

## EXAMPLE 5

Example 3 is repeated using magenta dye-forming 5-pyrazolone couplers 6 through 9 of U.S. Pat. 2,908,573 in place of the coupler used in Example 3. The results are similar to those obtained in Example 3.

## EXAMPLE 6

Example 3 is repeated using colored magenta dye-forming 5-pyrazolone couplers 1 through 5, 7 and 8 of U.S. Pat. 2,725,292, in place of the coupler used in Example 3. In this example the dye of the coupler remaining in the color processed layer as well as the magenta dye formed by coupler that coupled with oxidized color

developer during color processing are both stabilized against the destructive effects of prolonged exposure to light in the SANS fading test.

Similarly the valuable stabilizing effect of our stabilizing agents can be demonstrated for still other dyes particularly the dyes formed by chromogenic development of any of the known 5-pyrazolone couplers.

## EXAMPLE 7

10 A gelatinous silver halide emulsion is prepared as described by Trivelli and Smith in The Photographic Journal, page 330, May 1939. One portion of this emulsion is coated as a control identified as coating No. 1 on a cellulose acetate film support. Coating No. 2 is made of another portion of the emulsion to which our stabilizing compound No. 4 is added so that it is coated at a rate of 15  $10^{-4}$  mole (of stabilizer) per ft.<sup>2</sup>. Coating No. 3 is made of another portion of the emulsion to which our stabilizing compound No. 4 is added so that it is coated at the same rate as stabilizing compound No. 4. The coatings are given a sensitometric exposure and color developed in a conventional magenta color developing solution containing the color developing agent, 4-amino-N-ethyl-N-( $\beta$ -methanesulfonamidoethyl) - m - toluidine sesquisulfate 20 monohydrate, an alkali, an alkali metal sulfite and the magenta dye-forming coupler, 1-(2,4,6-trichlorophenyl)-3-(2,4-dichloroanilino)-5-pyrazolone (coupler No. 6 of U.S. Pat. 3,152,896). The color developed coatings are 25 then water washed, bleached in a conventional alkali metal ferricyanide-bromide bleach, fixed in a conventional alkali metal thiosulfate fixing bath washed and dried. Our stabilizer compounds 4 and 7 in coatings 2 and 3 impart 30 valuable protection to the magenta dye images as is illustrated by 3 weeks SANS test as described in Example 2. 35 Similar results are obtained when Example 7 is repeated with other dye-stabilizing compounds of our invention and with other primary aromatic amine color developing agents and other magenta dye-forming couplers including couplers 1, 2, 3, 4, 5, 7 and 8 of U.S. Pat. 40 3,152,896 as well as other diffusible magenta dye-forming couplers well known in the art.

Our stabilizer compounds are advantageously incorporated in the receiving layer of image receiving sheets to 45 stabilize the dye images transferred thereto. For example, image transfer dyes made from compounds I through XLVI of U.S. Pat. 3,227,551 and transferred to receiving layers containing our stabilizer compounds have improved 50 stability to prolonged exposure to light. Similarly, dye images produced from dye developers such as those described in U.S. Pat. 3,404,002 and transferred to receiving layers containing our stabilizer compounds are found to fade less upon prolonged exposure to light than the same images transferred to a receiving layer containing none of our stabilizers.

55 Similarly, the azo dye images produced in silver dye-bleach elements containing our stabilizers are substantially more stable to prolonged exposure to light than images that are not so protected. Thus our stabilizers are 60 advantageously incorporated in silver dye-bleach materials, such as those described in U.S. Patents 2,418,624, 2,420,630, 2,420,631, etc.

Our stabilizing compounds are also advantageously 65 incorporated in the azo dye image-forming layer of any of the diazo-type elements that are used for duplicating images. Thus our stabilizer compound is incorporated into the polymeric matrix layer containing the diazo salt(s) and coupler(s) where it advantageously protects the azo dye image produced upon development of the light image exposed layer.

In general the compounds of Formula I in which Z represents a



11

group are advantageously prepared by treating an enamine of the formula:

II



wherein  $R_1$ ,  $R_2$ ,  $R_6$  and  $R_7$  are as described previously with a quinone of the formula:

III



wherein  $R_3$ ,  $R_4$  and  $R_5$  are as described previously, according to the procedure described in Brannock et al. U.S. Pat. 3,184,457 issued May 18, 1965, incorporated herein as part of this application by reference. Compounds of Formula I in which  $Z$  represents an alkoxy group are advantageously prepared by reacting an enol ether compound of the formula:

IV



wherein  $R_1$ ,  $R_2$  and  $R_8$  are as described previously, with a quinone of Formula III in the presence of a Lewis acid catalyst as described in Brannock et al. U.S. Pat. 3,285,937 incorporated herein as part of this application by reference. The following table lists the compounds of Formulas II, III and IV that are used to form our illustrative compounds.

| Compound Number of— | Compound of Formulas II or IV                 | Compound of Formula III           |
|---------------------|-----------------------------------------------|-----------------------------------|
| Formula:            |                                               |                                   |
| 1                   | 1-morpholinoisobutylene                       | t-butylquinone.                   |
| 2                   | 1-(N'-ethoxycarbonyl-N-piperazino)isobutylene | Do.                               |
| 3                   | 1-(1'-piperidino)-2-ethylhex-1,2-ene          | Do.                               |
| 4                   | 1-(N-methylanilino)isobutene                  | t-octylquinone.                   |
| 5                   | 1-(N-butyylanilino)propene                    | Do.                               |
| 6                   | 1-(N-methylanilino)isobutene                  | Do.                               |
| 7                   | do                                            | t-butylquinone.                   |
| 8                   | 1-(3-ethoxycarbonyl-piperidino)isobutene      | Do.                               |
| 9                   | 1-(N-methylanilino)-2-butylhex-1,2-one        | t-octylquinone.                   |
| 10                  | do                                            | t-butylquinone.                   |
| 11                  | 1-(N-methylanilino)-2-ethylhex-1,2-ene        | t-octylquinone.                   |
| 12                  | 1-(N-hexyl-N-methylanilino)isobutene          | Do.                               |
| 13                  | 1-piperidinoisobutene                         | Do.                               |
| 14                  | 1-(N-methyl-N-octadecylamino)isobutene        | t-butylquinone.                   |
| 15                  | 1-(N-anilino)isobutene                        | 6-t-butoxy-2-methylquinone.       |
| 16                  | do                                            | 2-t-butyl-5-ethoxyquinone.        |
| 17                  | 1-(N-methylanilino)isobutene                  | 2-t-butyl-3-phenylquinone.        |
| 18                  | do                                            | 2-t-butyl-3-ethoxyquinone.        |
| 19                  | 1-(N,N-dimethylanilino)isobutene              | 1,2,3,4-tetrahydronaphthoquinone. |
| 20                  | Ethylisobutetyl ether                         | t-butylquinone.                   |
| 21                  | 1-(ethoxy)-2-ethylhex-1,2-ene                 | t-octylquinone.                   |
| 22                  | Ethyl isobutetyl ether                        | Do.                               |
| 23                  | Butyl isobutetyl ether                        | t-butylquinone.                   |
| 24                  | Octadecyl isobutetyl ether                    | Do.                               |
| 25                  | Docosyl isobutetyl ether                      | Do.                               |
| 26                  | 2-methylpentyl isobutetyl ether               | Do.                               |

The enamines of Formula II are advantageously prepared by the reaction of known secondary amines with known aliphatic aldehydes having at least one  $\alpha$ -hydrogen.

The enol ethers of Formula IV are derived from known aliphatic aldehydes having only one  $\alpha$ -hydrogen atom.

The quinones of Formula III are well known in the art and are either available or prepared by well known methods.

Our hydrophilic colloid layers containing dye images, such as, indophenol dye images, indoaniline dye images, azomethine dye images and azo dye images and a stabilizing amount of our nonalkyl-2-alkoxy-5-hydroxycoumarans provide a valuable technical advance in color image reproduction because these images are substantially more stable than the same images in layers containing no stabilizer or a prior art stabilizer.

The invention has been described in detail with particular reference to certain preferred embodiments thereof, but it will be understood that variations and modifications can be effected within the spirit and scope of the invention.

12

We claim:

1. A hydrophilic colloid layer containing a color photographic dye image, said layer containing at least one nondiffusible 5-hydroxycoumaran selected from the class consisting of a 2-amino-5-hydroxycoumaran and a 2-alkoxy-5-hydroxycoumaran.

2. A hydrophilic colloid layer containing a color photographic dye image, said layer containing at least one nondiffusible 5-hydroxycoumaran selected from the class consisting of those have the formula:



wherein  $R_1$  represents a member selected from the class consisting of hydrogen, an alkyl group, and the necessary atoms to complete with  $R_2$  a fully hydrogenated hydrocarbon ring having from 4 to 7 atoms in the ring;  $R_2$  represents a group selected from the class consisting of an alkyl group and the necessary atoms to complete with  $R_1$  a fully hydrogenated hydrocarbon ring having from 4 to 7 atoms in the ring;  $R_3$  represents a member selected from the class consisting of hydrogen, an alkyl group and an alkoxy group;  $R_4$  represents a member selected from the class consisting of hydrogen, an alkyl group, an alkoxy group and the necessary atoms to complete with  $R_5$  a saturated ring fused with the phenol ring;  $R_5$  represents a member selected from the class consisting of hydrogen, an

alkyl group, an alkoxy group, a mononuclear aryl group and the necessary atoms to complete with  $R_4$  a saturated ring fused with the phenol ring;  $Z$  represents a group selected from the class consisting of a

60



group and an  $-OR_8$  group;  $R_6$  represents a group selected from the class consisting of an alkyl group, an aryl group, a heterocyclic group having from 4 to 7 atoms in the ring and the necessary atoms to complete with  $R_7$  a heterocyclic ring having from 4 to 7 atoms in the ring;  $R_7$  represents a group selected from the class consisting of an alkyl group, an aryl group, a heterocyclic group having from 4 to 7 atoms in the ring and the necessary atoms to complete with  $R_6$  a heterocyclic ring having from 4 to 7 atoms in the ring; and  $R_8$  represents an alkyl group.

75

## 13

3. A hydrophilic colloid layer of claim 2 in which the Z group in the 5-hydroxycoumaran represents a



group wherein R<sub>6</sub> represents a group selected from the class consisting of an alkyl group, an aryl group, a heterocyclic group having from 4 to 7 atoms in the ring and the necessary atoms to complete with R<sub>7</sub> a heterocyclic ring having from 4 to 7 atoms in the ring; R<sub>7</sub> represents a group selected from the class consisting of an alkyl group, an aryl group, a heterocyclic group having from 4 to 7 atoms in the ring and the necessary atoms to complete with R<sub>6</sub> a heterocyclic ring having from 4 to 7 atoms in the ring.

4. A hydrophilic colloid layer of claim 2 in which the Z group in the 5-hydroxycoumaran represents a —OR<sub>8</sub> group in which R<sub>8</sub> represents an alkyl group.

5. A dye image-forming layer comprising a film-forming hydrophilic colloid layer containing at least one nondiffusible, 5-hydroxycoumaran selected from the class consisting of a 2-amino-5-hydroxycoumaran and a 2-alkoxy-5-hydroxycoumaran.

6. A dye image-forming layer of claim 5 in which the image-forming layer contains a silver halide emulsion.

7. A dye image-forming silver halide emulsion layer comprising a film-forming hydrophilic colloid layer containing at least one nondiffusible 5-hydroxycoumaran selected from those having the formula:



wherein R<sub>1</sub> represents a member selected from the class consisting of hydrogen, an alkyl group, and the necessary atoms to complete with R<sub>2</sub> a fully hydrogenated hydrocarbon ring having from 4 to 7 atoms in the ring; R<sub>2</sub> represents a group selected from the class consisting of an alkyl group and the necessary atoms to complete with R<sub>1</sub> a fully hydrogenated hydrocarbon ring having from 4 to 7 atoms in the ring; R<sub>3</sub> represents a member selected from the class consisting of hydrogen, an alkyl group and an alkoxy group; R<sub>4</sub> represents a member selected from the class consisting of hydrogen, an alkyl group, an alkoxy group and the necessary atoms to complete with R<sub>5</sub> a saturated ring fused with the phenol ring; R<sub>5</sub> represents a member selected from the class consisting of hydrogen, an alkyl group, an alkoxy group, a mononuclear aryl group and the necessary atoms to complete with R<sub>4</sub> a saturated ring fused with the phenol ring; Z represents a group selected from the class consisting of a



## 14

group and an —OR<sub>8</sub> group; R<sub>6</sub> represents a group selected from the class consisting of an alkyl group, an aryl group, a heterocyclic group having from 4 to 7 atoms in the ring and the necessary atoms to complete with R<sub>7</sub> a heterocyclic ring having from 4 to 7 atoms in the ring; R<sub>7</sub> represents a group selected from the class consisting of an alkyl group, an aryl group, a heterocyclic group having from 4 to 7 atoms in the ring and the necessary atoms to complete with R<sub>6</sub> a heterocyclic ring having from 4 to 7 atoms in the ring; and R<sub>8</sub> represents an alkyl group.

8. A dye image-forming silver halide emulsion layer of claim 7 in which R<sub>4</sub> represents the t-butyl group.

9. A dye image-forming silver halide emulsion layer of claim 7 in which R<sub>4</sub> represents the t-octyl group.

10. A magenta dye image-forming silver halide emulsion layer containing 3,3-dimethyl-5-hydroxy-2-(N-methylanilino)-6-t-octylcoumaran.

11. A magenta dye image-forming silver halide emulsion layer containing 2-(N-methylanilino)-6-t-butyl-3,3-dimethyl-5-hydroxycoumaran.

12. A magenta dye image-forming silver halide emulsion layer containing 2-(N-anilino)-6-t-butoxy-5-hydroxy-3,3,4-trimethylcoumaran.

13. A magenta dye image-forming silver halide emulsion layer containing 6-t-butyl-3,3-dimethyl-5-hydroxy-2-morpholino coumaran.

14. A magenta dye image-forming silver halide emulsion layer containing 6-t-butyl-3,3-dimethyl-2-(N'-ethoxy-carbonyl-N-piperazino)-5-hydroxycoumaran.

15. A magenta dye image-forming silver halide emulsion layer containing 6-t-butyl-3,3-dimethyl-2-(3-ethoxy carbonylpiperidino)-5-hydroxycoumaran.

16. In an element for color photography designed for dye image storage, said element comprising a support layer and at least one hydrophilic colloid layer for said dye image, the improvement comprising the use of a hydrophilic colloid layer containing a stabilizing amount of a nondiffusible, 5-hydroxycoumaran selected from the class consisting of a 2-amino-5-hydroxycoumaran and a 2-alkoxy-5-hydroxycoumaran for the said dye image.

## References Cited

## UNITED STATES PATENTS

|    |           |         |                 |           |
|----|-----------|---------|-----------------|-----------|
| 45 | 2,272,191 | 2/1942  | Fierke          | 96—74     |
|    | 2,274,551 | 2/1942  | Kenyon et al.   | 260—152   |
|    | 2,984,568 | 5/1961  | Hart et al.     | 96—84     |
|    | 2,535,058 | 12/1950 | Gleim et al.    | 44—63     |
| 50 | 3,184,457 | 11/1966 | Brannock et al. | 260—247.7 |
|    | 3,285,937 | 11/1966 | Brannock et al. | 260—346.2 |
|    | 3,432,300 | 3/1969  | Lestine et al.  | 96—74     |

NORMAN G. TORCHIN, Primary Examiner

A. T. SURO PICO, Assistant Examiner

U.S. Cl. X.R.

96—77